

Jan. 9, 1951

G. MOHLING ET AL  
VALVE AND TURBINE STEELS

2,537,477

Filed Jan. 15, 1947



INVENTOR

Guenther Mohling  
Thomas G. Wilson  
By Green, McCallister & Miller  
Their Attorneys

## UNITED STATES PATENT OFFICE

2,537,477

## VALVE AND TURBINE STEELS

Gunther Mohling, Loudonville, and Thomas Y. Wilson, Albany, N. Y., assignors to Allegheny Ludlum Steel Corporation, a corporation of Pennsylvania

Application January 15, 1947, Serial No. 722,118

8 Claims. (Cl. 75—128)

1

The present invention pertains to high temperature steels of moderate strength, generally, lower alloy content and, incidentally, lower cost. The strength at heat of these alloys is, however, considerably higher than that of commercial alloys in use at the beginning of World War II.

Two previous patents of Gunther Mohling, Numbers 2,373,490 and 2,397,034, deal with alloys of maximum strength at high temperatures, the utilizations of which were mainly confined to gas turbines for military aircraft.

There is a wide field for use of alloys of our invention, for instance, improved valves for internal combustion engines, improved steam turbine buckets and gas turbine buckets for the low temperature stages of multi-stage turbines.

There has been a continuous demand for improved alloys that may be used in this general field and an increased demand for less expensive alloys. It will be appreciated that steels or alloys used in connection with internal combustion engines are subjected to considerable temperature variations and to relatively high temperatures, at least periodically. Steels used for turbines are also subjected to considerable temperature variations and to relatively high temperatures during their utilization. Such steels must, thus, have special physical, structural, and other qualities such that they will withstand the temperature conditions encountered, will have a reasonable period of life, and will also have resistance to corrosion under service conditions. For example, in combustion engines, lead ethyl bromides are extremely corrosive, and although in turbine utilization the steam or gases are not as highly corrosive, they are strongly corrosive due to the temperature at which the parts are utilized.

Steels for turbines, such as herein contemplated, should be capable of withstanding temperatures from about 900° to 1350° F., while valve steels should be capable of withstanding temperatures from about 1000° to 1400° F.

It will be apparent that steels or alloys such as herein considered, should have a high resistance to the normal corrosive action of combustion fluids and exhaust gases of internal combustion engines and to the high temperature gases employed in turbine utilizations. They should have high resistance to deformation at the temperatures involved and while being subjected to stress and wear conditions. Adequate hardness must be maintained at a temperature as high as about 1400° F. and after prolonged exposure to continuous or intermittent application thereof.

In connection with turbine utilizations, the steels should have good damping capacity. They

2

should have enough or sufficient ductility that the parts will give some warning before they give way entirely, near the end of their normal period of life.

All steels herein considered, when made in accordance with our invention, have improved common characteristics, such as better corrosion resistance at high temperature without an excessive loss of strength; that is, they have better oxidizing resistance for any temperature of the operating range. They are also less expensive than steels of comparable strengths since they make possible the utilization of smaller percentages of the strategically critical elements, such as molybdenum, tungsten and columbium.

It has thus been an object of our invention to provide new and improved steels for high temperature utilizations.

Another object has been to provide high temperature steels that may successfully utilize lower percentages of the more expensive alloying elements.

Another object has been to provide high temperature alloy steels that may be used as cast, forged or machined engine valves and turbine vanes or buckets.

These and many other objects of our invention will appear to those skilled in the art from the description thereof, the claims and the exemplary illustrations.

In the drawings:

Figure 1 is a perspective view in elevation of a typical metal valve 10 utilizing steel of our invention;

Figure 2 is a perspective sectional view of a typical turbine wheel 15 having metal buckets or vanes 16 utilizing steel of our invention.

Table I gives the analysis of a number of melts which are in the preferred composition range of our present invention. Common to all these melts is the simultaneous presence of molybdenum, tungsten and columbium in the range of about 2 to substantially less than 6 percent total and of a minimum total of about 1.20 percent.

The carbon content of all melts is below about 1 percent. Chromium is present from about 12 to 26 percent and nickel between about 3 to 20 percent. It is common knowledge that the alloys of chromium and nickel are mostly ferritic or magnetic if the nickel content is somewhat below 7 percent. These alloys will be useful in the lower end of the temperature range, that is up to about 1100° F. If the nickel content is substantially above 7 percent the alloy becomes a stable austenite and may be used in the higher end of the temperature range. Three exemplary melts con-

tain up to 20% of cobalt. These may be used if a somewhat higher strength and hot hardness is required and the application warrants the extra cost.

Manganese and silicon may be present up to about 2.50 percent; while they are not essential elements in an alloy of our invention, they may be present in usual commercial amounts. A certain amount of silicon is usually present due to its appearance in other ferroalloys used in making the alloying additions. Nitrogen, although not essential, may be present up to about .25 percent; additions to the melt may be accomplished for this purpose.

In addition to other beneficial effects, proper amounts of nickel insure a stable steel under conditions of service and proper amounts of chromium insure corrosion resistance. Cobalt (not essential) may be used to produce beneficial effects such as hot hardness and strength. The carbon content is maintained below about 1% and is preferably kept about or below .60%.

The alloys of our invention may contain normal amounts of other alloying elements in such quantities as to not alter desired properties of the alloy. That is, some additional alloying element or elements may be added without changing the essential characteristics of the alloy. "Remainder substantially iron" as herein employed means that the alloy may contain percentages of additional non-ferrous alloying elements of such nature and quantity as to not destroy the basic improved properties of the alloy.

Table II shows a number of time to rupture tests on these melts, in which a heat treated or cast test piece was subjected to a constant load at temperatures of 1000, 1100, 1200, 1350 and 1500° F. The life in hours until failure is given, together with the elongation and reduction in area is in percent of original. The double heat treatment given to each test piece is described in the Mohling Patent #2,401,580 of June 4, 1946.

Table III shows rupture properties of two commercial steels, #1 a prominent automotive valve steel and #2 an aircraft exhaust valve steel. #1 is a chromium-nickel alloy containing about 3 percent of molybdenum; #2 a chromium-nickel alloy containing about 3 percent of tungsten. U-34 is the same alloy as #2 in which the tung-

sten is replaced with 1½ percent of molybdenum, 1 percent of tungsten and .50 percent of columbium according to our invention.

It is evident from comparison of Tables II and III that the properties of all alloys in Table II (see also U-34 of Table III) are very far superior to the commercial alloys in Table III. For example, the life of U-34 at 1500° F. is about three times that of steel #2, see Table III. Steel #1 of Table III may be compared, for example, with steels S-921 and S-931 of Table II.

What we claim as new according to our invention are alloys for intermediate high temperature service, which fall in substantially the following ranges of composition:

|            |       |                                        |
|------------|-------|----------------------------------------|
| Carbon     | ..... | 0.5-1.00%                              |
| Silicon    | ..... | 2.50% maximum                          |
| Manganese  | ..... | 20-2.50%                               |
| Chromium   | ..... | 12-30%                                 |
| Nickel     | ..... | 3-20%                                  |
| Molybdenum | ..... | 5.0-2.00%                              |
| Tungsten   | ..... | 5.0-2.00%                              |
| Columbium  | ..... | 5.0-2.00% (may be as low as about 20%) |

The total of the last three elements being less than 6%, and preferably, within a maximum of about 4.5%, see Table I.

With or without cobalt.

Remainder iron, or substantially iron with or without some nitrogen.

TABLE I  
*Analyses of experimental melts*

| Heat No.     | C   | Mn   | Si  | Cr    | Ni    | Co    | Mo   | W    | Cb   |
|--------------|-----|------|-----|-------|-------|-------|------|------|------|
| S-673        | .37 | .59  | .61 | 19.94 | 13.69 | ..... | 1.18 | 1.20 | 1.92 |
| S-764        | .39 | .58  | .56 | 20.74 | 10.66 | ..... | 1.16 | 1.03 | 1.96 |
| S-784        | .39 | 1.54 | .35 | 18.80 | 3.17  | ..... | .90  | 1.23 | 1.05 |
| S-920        | .56 | 1.62 | .42 | 17.84 | 4.12  | ..... | 1.09 | .95  | 1.09 |
| S-921        | .55 | 1.59 | .42 | 20.10 | 4.10  | ..... | 1.14 | .99  | 1.12 |
| S-921 (Cast) | .60 | 1.20 | .47 | 26.29 | 4.19  | ..... | 1.13 | .94  | .72  |
| S-931        | .37 | 1.59 | .40 | 18.65 | 4.06  | ..... | 1.13 | .95  | 1.09 |
| S-932        | .52 | 1.59 | .45 | 18.41 | 4.08  | ..... | .89  | .95  | 1.09 |
| S-967        | .47 | 1.31 | .40 | 20.56 | 4.00  | ..... | 1.13 | 1.28 | .24  |
| U-34         | .36 | .55  | .36 | 13.63 | 13.73 | ..... | 1.59 | .97  | .55  |
| U-39         | .35 | .60  | .43 | 23.27 | 13.81 | ..... | 1.52 | .88  | .54  |
| U-73         | .36 | .44  | .50 | 21.92 | 13.81 | 19.20 | 1.58 | 1.09 | .55  |
| U-88         | .41 | .46  | .44 | 23.90 | 9.66  | 14.47 | 1.58 | 1.00 | .57  |
| U-89         | .41 | .50  | .53 | 24.19 | 9.76  | 10.42 | 1.60 | 1.12 | .53  |
| U-247        | .44 | 1.52 | .39 | 18.00 | 4.10  | ..... | 1.13 | 1.17 | .99  |
| U-268        | .37 | 1.18 | .44 | 18.35 | 4.22  | ..... | 1.03 | .94  | 1.12 |

50

TABLE II

*Time-to-rupture tests*

| Heat No. | Heat Treatment                    | Load, P. s. i.               | Time, Hours             | Elongation, Per Cent | Reduction, Per Cent | Hot Brinell at 1400° F. |
|----------|-----------------------------------|------------------------------|-------------------------|----------------------|---------------------|-------------------------|
| 1000° F. |                                   |                              |                         |                      |                     |                         |
| S-921    | As Cast                           | { 60,000<br>50,000<br>40,000 | { 441<br>1,181<br>3,097 | { 5.6<br>3.4<br>5.0  | { 8.8<br>8.8<br>8.7 |                         |
| U-247    | 2150° 30 min. W + 1100° 16 hrs. A | 50,000                       | 2,809                   | 7.8                  | 14.2                |                         |
| U-268    | do                                | { 60,000<br>50,000           | { 1,168<br>1,598        | { 9.6<br>5.2         | { 9.4<br>5.8        |                         |
| 1100° F. |                                   |                              |                         |                      |                     |                         |
| S-921    | As Cast                           | { 50,000<br>40,000           | { 73<br>1,033           | { 2.9<br>2.0         | { 11.3<br>3.3       |                         |
| U-247    | 2150° 30 min. W + 1100° 16 hrs. A | { 60,000<br>50,000<br>40,000 | { 66<br>416<br>1,758    | { 8.2<br>5.5<br>3.1  | { 9.4<br>7.0<br>5.2 |                         |

TABLE I...Continued

## Analyses of experimental melts—Continued

| Heat No. | Heat Treatment   | Load, P. S. I. | Time, Hours | Elongation, Per Cent | Reduction, Per Cent | Hot Brinell at 1400° F. |
|----------|------------------|----------------|-------------|----------------------|---------------------|-------------------------|
| 1200° F. |                  |                |             |                      |                     |                         |
| S-931    | 2150° 30 min. W+ | 30,000         | 1,058       | 4.0                  | 4.8                 |                         |
|          | 1200° 16 hrs. A. | 25,000         | 5,078       | 6.9                  | 4.0                 |                         |
| S-764    | 2150° 1 hr. W+   |                |             |                      |                     |                         |
|          | 1400° 16 hrs. A. | 25,000         | 7,442       | 9.0                  | 5.6                 |                         |
| S-920    | 2150° 1 hr. W+   | 30,000         | 152         | 18.0                 | 22.0                |                         |
|          | 1400° 16 hrs. A. | 20,000         | 3,254       | 4.0                  | 2.4                 |                         |
| S-921    | do               | 30,000         | 208         | 13.5                 | 13.0                |                         |
|          |                  | 25,000         | 731         | 10.0                 | 9.0                 |                         |
|          |                  | 20,000         | 2,695       | 5.0                  | 3.0                 |                         |
| S-931    | do               | 30,000         | 372         | 6.0                  | 4.0                 |                         |
| S-932    | do               | 30,000         | 232         | 7.0                  | 3.5                 |                         |
| S-967    | do               | 30,000         | 315         | 7.0                  | 6.0                 |                         |
|          |                  | 25,000         | 837         | 10.5                 | 6.2                 |                         |
| 1350° F. |                  |                |             |                      |                     |                         |
| S-673    | 2150° 1 hr. W+   | 20,000         | 221         | 12.5                 | 12.8                |                         |
|          | 1400° 16 hrs. A. | 20,000         | 279         | 10.0                 | 7.0                 |                         |
| S-920    | do               | 25,000         | 41          | 25.0                 | 24.0                |                         |
| S-921    | do               | 20,000         | 243         | 11.5                 | 16.0                |                         |
| S-931    | do               | 20,000         | 665         | 17.0                 | 16.0                |                         |
| S-932    | do               | 20,000         | 297         | 19.0                 | 17.0                |                         |
| S-967    | do               | 20,000         | 420         | 7.0                  | 6.0                 |                         |
| 1500° F. |                  |                |             |                      |                     |                         |
| S-673    | 2150° 1 hr. W+   | 12,500         | 91          | 8.0                  | 9.0                 |                         |
| S-764    | do               | 12,500         | 106         | 3                    | 3                   |                         |
| U-39     | do               | 10,000         | 84          | 4.0                  | 5.0                 | 128                     |
| U-89     | do               | 10,000         | 166         | 2.0                  | 2.0                 | 156                     |
| U-88     | do               | 10,000         | 299         | 3.0                  | 1.0                 | 156                     |
| U-73     | do               | 10,000         | 280         | 2.0                  | 1.0                 | 156                     |

<sup>1</sup>This means 1 hour temperature treatment at 2150° F. followed by a water quench. The second part of the heat treatment is at 1400° F. for 16 hours followed by air cooling. The same interpretation applies to the other heat treatments set forth.

TABLE III  
Time-to-rupture tests on commercial valve steels

|                                                                    | Load, p. s. i. | Time, Hours | Elongation, Per Cent | Reduction, Per Cent |    |
|--------------------------------------------------------------------|----------------|-------------|----------------------|---------------------|----|
| 1200° F.                                                           |                |             |                      |                     |    |
| Steel #1                                                           | 25,000         | 148         | 20                   | 34                  | 50 |
|                                                                    | 20,000         | 375         | 34                   | 27                  |    |
| Steel #2                                                           | 25,000         | 48          | 25                   | 30                  |    |
|                                                                    | 20,000         | 168         | 38                   | 37                  |    |
| 1350° F.                                                           |                |             |                      |                     |    |
| Steel #1                                                           | 20,000         | 9           | 46                   | 47                  | 55 |
| Steel #2                                                           | 20,000         | 95          | 5                    |                     |    |
| 15,000° F.                                                         |                |             |                      |                     |    |
| Steel #1                                                           | 7,000          | 13          | 76                   | 57                  | 60 |
| Steel #2                                                           | 10,000         | 139         | 3                    | 2                   |    |
| U-34 (Same steel as steel #2, modified according to our invention) | 10,000         | 334         | 3                    | 4                   |    |

It will be apparent that various modifications, omissions, and additions may be made and that various alloys may be produced within the broader ranges without departing from the spirit and scope of our invention as indicated by the appended claims.

What we claim is:

1. An improved, inexpensive, heat resistant alloy that will withstand temperature variations and that has a better corrosion resistance at high temperatures without an excessive loss of

strength, said alloy containing below about 1% carbon, about 12-26% chromium, about 3-20% nickel, molybdenum, tungsten, and columbium in a minimum total amount of about 1.2% and up to a total amount of substantially less than 6%, and the remainder iron; all of the named elements as its essential elements, with usual commercial amounts of the elements manganese and silicon.

2. An improved, inexpensive, heat resistant alloy that will withstand temperature variations and that has a better corrosion resistance at high temperatures without an excessive loss of strength, said alloy containing below about 1% carbon, about 12-30% chromium, about 3 to 7% nickel, the elements molybdenum, tungsten, and columbium in a total minimum amount of about 1.2% and up to a total amount of substantially less than 6%, up to about 2.5% of each of the elements manganese and silicon, up to about .25% nitrogen, up to about 20% cobalt, and the remainder substantially iron; the essential elements being carbon, chromium, nickel, molybdenum, tungsten, columbium and iron; the carbon, chromium, nickel, molybdenum, tungsten, and columbium being essential in the proportions stated.

3. An improved, inexpensive, essentially ferritic-magnetic, heat resistant alloy that will withstand temperature variations and that has a better corrosion resistance at high temperatures without an excessive loss of strength, said alloy containing below about 1% carbon, about 12-26% chromium, about 3-7% nickel, the elements molybdenum, tungsten and columbium in

a total amount of not less than about 1.2% and up to a total amount of substantially less than 6%, up to about 2.5% of each of the elements manganese and silicon, up to about .25% nitrogen, up to about 20% cobalt, and the remainder substantially iron; the essential elements being carbon, chromium, nickel, molybdenum, tungsten, columbium, and iron.

4. An improved, inexpensive, heat resistant austenitic alloy that will withstand temperature variations and that has a better corrosion resistance at high temperatures without an excessive loss of strength, said alloy containing below about 1% carbon, about 12-26% chromium, about 7-20% nickel, the elements molybdenum, tungsten, and columbium in a total minimum amount of not less than about 1.2% and up to a total amount of substantially less than 6%, up to about 2.5% of each of the elements manganese and silicon, up to about .25% nitrogen, and the remainder iron; the essential elements being carbon, chromium, nickel, molybdenum, tungsten, columbium and iron.

5. An improved, inexpensive, heat resistant alloy that will withstand temperature variations and that has a better corrosion resistance at high temperatures without an excessive loss of strength, said alloy containing carbon within the range of about .05-1%, about 12-30% chromium, about 3-20% nickel, about .50-2% of each of the elements molybdenum and tungsten, about .20-2% columbium; the molybdenum, tungsten, and columbium being in a maximum total amount of substantially less than 6%, about .20-2.5% manganese, up to about 2.5% maximum silicon, up to about .25% nitrogen, and the remainder iron; the elements carbon, chromium, nickel, molybdenum, tungsten and columbium being essential in the proportions stated.

6. A heat resistant article suitable for operation within a temperature range of 900-1400° F. made from an alloy as defined in claim 5.

7. An improved, inexpensive, heat resistant alloy that will withstand temperature variations and that has a better corrosion resistance at high temperatures without an excessive loss of strength, said alloy containing below about 1% carbon, about 12 to 30% chromium, about 3 to

20% nickel, the elements molybdenum, tungsten and columbium in a total minimum amount of about 1.2% and up to a total amount of substantially less than 6% and in substantially equal proportions, up to about 2.5% of each of the elements manganese and silicon, up to about .25% of nitrogen, and the remainder iron; the essential elements being carbon, chromium, nickel, molybdenum, tungsten and columbium in the proportions stated.

8. An improved, inexpensive, essentially ferritic-magnetic, heat resistant alloy that will withstand temperature variations and that has a better corrosion resistance at high temperatures without an excessive loss of strength, said alloy containing below about 1% carbon, about 12 to 30% chromium, about 3 to 7% nickel; molybdenum, tungsten and columbium in a minimum total amount of about 1.2% and up to a total amount of substantially less than 6%, and the remainder substantially iron; the essential elements being carbon, chromium, nickel, molybdenum, tungsten, columbium and iron; and, with usual commercial amounts of the elements manganese and silicon.

GUNTHER MOHLING.  
THOMAS Y. WILSON.

#### REFERENCES CITED

30 The following references are of record in the file of this patent:

#### UNITED STATES PATENTS

| Number       | Name        | Date          |
|--------------|-------------|---------------|
| 35 2,229,065 | Franks      | Jan. 21, 1941 |
| 2,397,034    | Mohling     | Mar. 19, 1946 |
| 2,398,702    | Fleischmann | Apr. 16, 1946 |
| 2,416,515    | Evans       | Feb. 25, 1947 |
| 2,429,800    | Briggs      | Oct. 28, 1947 |
| 40 2,432,615 | Franks      | Dec. 6, 1947  |

#### OTHER REFERENCES

Progress Report on "Heat Resisting Metals for Gas Turbine Parts" (N-102), P. B. 39579; by the 45 War Metallurgy Division, National Research Defense Committee. Published September 21, 1943; declassified February 18, 1946.